

## UNITED STATES PATENT OFFICE

FRITZ STEINBERG, OF BARMEN-LANGERFELD, GERMANY, ASSIGNEE TO AMERICAN BEMBERG CORPORATION, OF NEW YORK, N. Y., A CORPORATION OF DELAWARE

METHOD OF EQUALIZING THE COLOR EFFECT OF COTTON YARN TO THAT OF CUPRAMMONIUM SILK

No Drawing. Application filed November 26, 1930, Serial No. 498,439, and in Germany November 25, 1929.

In dyeing material which is composed partly of two different materials, for example, cotton and cuprammonium (Bemberg) yarn used in hosiery, etc., it has been noticed that the cotton portion takes on a decidedly lighter shade when dyed than the cuprammonium or Bemberg portion. This effect has been particularly noticeable in hosiery dyeing, where the toes and heels, of cotton, are lighter in color than the remainder of the article. Formerly this necessitated the dyeing of the cotton and cuprammonium portions separately before making the hosiery.

The method last outlined, obviously, has many disadvantages, as it is inefficient, expensive, and the risk of having the cuprammonium fabric damaged. Furthermore, artificial filaments when so dyed and knitted are not as resistant, and may not be wet treated as well as the cotton.

The object of this invention is to eliminate these disadvantages arising from the varying hues presented when a composite yarn is dyed. This is accomplished by previously treating the cotton yarn in a manner similar to that applied to artificial silk. Therefore, the cotton, made up into a strand, is treated with a copper ammonia solution. This produces a slight swelling and loosening of the filaments while the copper ammonium caustic is being absorbed. The cotton yarn is later treated in order to remove the copper contained in the filaments. The yarn is then passed through several washings until a neutral reaction occurs, or is reached, and the yarn is dried. It is advantageous to apply tension to the yarn during these treatments in order to avoid shrinkage.

For practical reasons this treatment may be divided into a pre-treatment with a diluted solution and a post-treatment wherein a somewhat stronger solution is used, and whereby the solution first used for post-treatment may be later used for the pre-treatment since the copper content decreases with the use of the solution.

The object of the pre-treatment is mainly to wet the cotton in order to insure a uniform absorption of the solution in the subsequent post-treatment. The application of tension

is, ordinarily, not necessary in the pre-treatment, although some tension will lessen the danger of a minor shrinkage.

This treatment imparts to the cotton yarns the same dyeing affinity as is found in the cuprammonium silk, and will offset the disadvantages found hitherto, and enumerated supra.

The method may be more clearly seen from a study of the following example:

The cotton is subjected, first, to a pre-treatment with a wetting alkaline solution made from a previously used post-treatment solution. To obtain this solution, the used solution containing 0.53-0.58 percent of copper is diluted by water until a copper content of 0.39-0.40 results. The ratio of the textile material to the bath is 1:20 for this pre-treatment wetting caustic solution.

As the etching caustic or post-treatment solution a copper ammonium solution containing from 0.70-0.75 percent copper and 17-20 percent ammonia is employed. This may be prepared by dissolving the corresponding quantity of copper in concentrated ammonia, so that a copper content of from 1.1-1.3 percent copper is obtained. This solution is then diluted with a used solution until a copper content of 0.70-0.75 results. The proportion of textile material to the solution is 1:14.5.

Subsequently to this treatment, a further treatment with an ammoniacal ammonium sulphate is used in order to remove the copper. In order to prepare this solution 2.5 liters of ammonia of a specific weight of 0.901 and 0.5 liters of sulphuric acid of a specific gravity corresponding to 60° Bé. are dissolved in 100 liters of water. The ratio of textile material to the solution is 1:30.

After this treatment, the cotton is acidified in a bath of from 1-1.5 percent sulphuric acid and rinsed twice in water. Extracting and drying follow.

To obtain the necessary tension for the various stages of the treatment, primarily for the concentrated solution and the ammonium sulphate treatment, but also for the wetting, mercerizing machines may be advantageously employed. By this means the

55

60

65

70

75

80

85

90

95

100

yarn is either completely immersed or the liquid for the treatment is applied between the rolls of the mercerizing machine by means of pipes. The liquids used in treating the yarn may be applied several times by use of a circular pumping system, and thereby a more uniform effect may be obtained.

Having now fully disclosed my invention as required by the patent statutes, what I claim is:

- 10 1. In a method for equalizing the dyeing effect of a fabric comprising a mixture of cotton and cuprammonium yarn, the step of treating the cotton with a copper-oxide-ammonia solution.
- 15 2. In a method as outlined in claim 1, in which a subsequent treatment with ammonium sulphate is employed prior to the dyeing step.
- 20 3. In a method for equalizing the dyeing effect of a textile comprising a mixture of cotton and cuprammonium yarn, the steps of treating the cotton yarn with a copper oxide ammonia solution, an ammonium sulphate solution and then washing and drying, in successive steps.
- 25 4. A method for equalizing the dyeing effect of a textile material comprising a mixture of cotton and cuprammonium silk, wherein the cotton is first treated with a bath containing 0.39 to 0.40 percent copper, then with a bath containing 0.70 to 0.75 percent copper, then with an ammonium sulphate bath, and subsequently washed and dried.
- 30 5. In testimony whereof I affix my signature.

FRITZ STEINBERG.